

## UNITED STATES PATENT OFFICE

2,573,882

METAL COATING PROCESS AND OIL FINISH-  
ING COMPOSITION THEREFORGeorge W. Waters, Wood River, Ill., assignor to  
Shell Development Company, San Francisco,  
Calif., a corporation of DelawareNo Drawing. Application April 12, 1947,  
Serial No. 741,001

22 Claims. (Cl. 117—51)

1

This invention relates to metal coating or alloying of metals. More particularly this invention pertains to oil compositions used in tinning, terne coating, lead coating and the like in order to facilitate and aid in coating or alloying a base metal with a uniform and tenacious metal coating.

This process for example, the tinning process comprises essentially coating base metals by dipping and the like said metals into a bath of molten tin thereby coating the base metal with a thin film of metallic tin. The tinning process is carried out at elevated temperatures and when skillfully done with the aid of good fluxing agents and proper tinning oils actually forms an alloy of tin and the metal being treated which is generally iron, steel and other ferrous metals.

To insure strong adherence of the tin to the metal surface being coated, the metal must be absolutely clean and free of any grease, dirt, oxide film and rust. This is necessary to insure intimate contact of the metal with the molten tin, terne composition and the like. Metals which are to be coated with tin and the like are therefore carefully prepared by being properly mechanically and chemically treated, pickled and kept in slightly acidic solution in order to prevent oxidation of the metal surface prior to entering the tinning bath or the like.

Briefly stated, for example, one method of tin coating of base metals comprises dipping or passing a properly cleaned metal into a bath of molten tin, on to an oil bath and then through cleaners to remove excess oil and polish the tinned metal surface. The general procedure is to pass a mildly pickled metal plate from a slightly acidified storage tank into a tin pot usually divided into a series of compartments. Each compartment contains a series of rollers through which the metal can pass during its various stages of tin coating. The molten tin occupies the lower or bottom part of the tin pot. On the feed end of the pot floats a layer of flux and on the exit end floats a much deeper layer of oil.

The flux serves to give final preparation of the metal surface before being immersed into the molten tin. It consists generally of zinc chloride or mixtures of zinc chloride and sodium chloride or ferric chloride or ammonium chloride and the like. The function or purpose of the flux is to clean thoroughly the metal surface, remove moisture, absorb any oxide film, pickling scum and control more or less the wettability of the metal by the tin so that the molten tin would react and adhere uniformly and tenaciously to the metal surface treated.

2

From the fluxing bath the metal proceeds on through a series of rollers through a molten tin bath kept at a temperature of between about 525° F. to above about 800° F. and preferably between about 530° and about 560°, depending upon the operating conditions. The tinned metal then proceeds through an oil bath while passing through rollers where excess tin is removed, better distribution of the tin coating is secured and oxidation of the tin is inhibited. The tinned metal having a thin film of oil on it proceeds on out of the oil bath and receives a cleaning treatment where excess oil is removed. Any remaining oil left on the metal aids in polishing the metal to a desired surface finish.

Articles of odd shape can be tin coated by mechanical or hand dipping into a flux coating tin pot and then redipped into an oil coated tin pot which on withdrawal come in contact with the oil and receives its beneficial treatment. If desired, the metal can then be immersed into a hot oil bath for final oil treatment in order to control more closely the thickness of the tin coating and also such oil treatment acts to some degree as a quenching medium.

Tinning oils play a vital role in the tinplating art for they serve to secure better distribution of tin on the base metal being coated, aid in removal of excess tin and protect the tin from oxidation or discoloration while being cooled. To accomplish these and other features a good tinning oil must be capable of absorbing oxides so as to keep the metal surface clean; it must have a suitable interfacial tension with molten tin and with the atmosphere and it must be stable and not tend to deteriorate or polymerize even after long periods of use under extremely high temperatures. Efficient tinning oils should in addition form a uniform film on the coated metal surface while in the tin pot but on emerging from the pot drain off easily and quickly. Oils which do not drain off easily must be continuously replaced which is quite an expense. Such oils may also tend to form globules or isolated patches on the tinned surface which produce depressions on the tin coating, resulting in localities which are very thin and which form grease marks on the tinned surface.

One main criterion of a good tinning oil as stated above is its ability to drain off rapidly from the tinned article as it emerges from the hot oil bath. From this aspect straight mineral oils and even palm oil after relatively short periods of use are not satisfactory. This desirable phenomenon of rapid draining seems to be associated with the presence of certain polar bodies

in the oil. An oil containing a plurality of these polar bodies drains off rapidly and leaves the tinned surfaces clean and bright. It is assumed that such oil films tend to form one or more aggregates which move continuously over the surface in an apparently random fashion. As the activity of the aggregates becomes reduced owing to reduction of these polar bodies, the draining of the oil is reduced and eventually a "continuous film" state is reached where the draining properties of oils are considerably retarded and the oil is no longer suitable for use. It is postulated that the efficiency of such oils is due to the formation of a monomolecular absorbed layer over the surface of the tin.

Generally oils used in tinplating are subjected to elevated temperatures of at least 460° F. and higher for long intervals. It is therefore essential that such oils be chemically stable at such temperature, without undue volatilization, decomposition or polymerization.

Palm oil is known to be an efficient tinning oil. However, it has several serious drawbacks in that it is costly, difficult to obtain and above all polymerizes readily at temperatures about 470° F. resulting in sludging and high oil losses. Also other beneficial tinplate properties of palm oil are destroyed at temperatures above 470° F. At this elevated temperature palm oils leave on the tinplate streaks of oil resulting in a dull, lustreless coated surface.

It is an object of this invention to produce an excellent tinning oil having a petroleum hydrocarbon base. Another object of this invention is to produce a new and improved tinning oil which is stable at extremely high temperatures for long periods of time. Another object of this invention is to produce a new and improved tinning oil having the ability to take up oxide, to readily absorb flux residue and to promote the spreading of tin and other molten metals. Still another object of this invention is to produce a tinning oil which does not stain or have bad effects on the coated surface if left on. Furthermore, it is another object of this invention to produce a tinning oil which drains and cleans easily and which is not a fire hazard.

The above and other objects may be attained in accordance with the present invention by admixing with a mineral oil base containing a minor amount of a high boiling nitrogen-containing organic compound or mixtures of nitrogen-containing organic compounds, a suitable amount of hydrogenated animal, vegetable, marine oils, distillate and residuum fractions of said oils and mixtures of said oils and/or their fractions.

Among the hydrogenated animal, vegetable and marine oils and their fractional derivatives which can be used for metal coating compositions of this invention are:

#### I. Animal oils

Tallow (beef, mutton, goat, etc.) oils  
Lard oil  
Bone oil  
Neat's-foot oil  
Wool fat  
Horse foot oil, etc.

#### II. Vegetable oils

##### A. Non-drying oils

Castor oil, cashew nut oil, peanut oil, cocoanut oil, jojoba seed oil, olive oil, olive kernel oil, palm oil, palm kernel oil, etc.

##### B. Semi-drying oils

Corn oil, cottonseed oil, kapok oil, rapeseed oil, ravicon oil, sesame oil, sunflower oil, teaseed oil, rice bran oil, etc.

##### C. Drying oils

Linseed oil, oiticica oil, perilla oil, soybean oil, tung oil, poppyseed oil, hempseed oil, etc.

#### 10 III. Marine and fish oils

Codfish oil, codliver oil, dogfish oil, dolphin body oil, dolphin fish oil, herring oil, Japfish oil, menhaden oil, porpoise body and jaw oils, salmon oil, sardine and sardine liver oils, seal oil, shark and shark liver oils, sperm whale body and head oils, whale oil, etc.

#### IV. Hydrogenated residuum fractions obtained from oils listed under Groups I, II, and III.

#### 20 V. Hydrogenated distillate fractions obtained from oils listed under Groups I, II, and III.

Hydrogenation of any of the above oils, their

distillate and residuum fractions and/or their mixtures can be carried out by any convenient method but preferably under such conditions as in the presence of steam and a suitable catalyst so that the resultant hydrogenated product is acidic. The hydrogenated product should be added to a mineral oil base containing a nitrogen-containing organic compound in amount sufficient to maintain the acid number of the tinning or metal coating oil composition at not less than 3 and not above about 15, and preferably between about 4 to 10. In order to maintain the acid number of the composition at approximately these values, a replenishing agent is added to the oil composition during use. The replenishing agent comprises a concentrate of mineral oil and hydrogenated fatty oil and/or fractions of

30 hydrogenated fatty oils such as the hydrogenated distillate or residuum fractions made up in a ratio varying from 1:3 to about 3:1 parts by weight of each ingredient respectively and preferably the replenishing concentrate is made up of equal parts by weight of mineral oil and the hydrogenated fatty product. The replenishing concentrate is added in amounts sufficient to adjust the acid number of the base composition to not less than about 3 and not above about 15.

35 The amount of organic nitrogen containing compound used to stabilize the composition against oxidation deterioration and the like varies from between about 0.25 to 2.0% and preferably between about 0.5 to 1.0% by weight.

40 55 Of the hydrogenated fatty oils and their fractions enumerated above, the preferred tin and metal coating additives are the hydrogenated fish and/or marine oil distillates and their mixtures. The fish and/or marine oil distillate products

50 can be recovered from such oils by any conventional means and then hydrogenated or the oil can be hydrogenated first and the product then split and the overhead distillate fraction removed by distillation, extraction and the like.

60 65 For example, a fish oil such as herring oil, menhaden oil and the like, can be hydrogenated and split and subsequently distilled to produce an overhead distillate of hydrogenated fish oil. Another preferred fatty oil fraction is obtained by splitting the above hydrogenated fish oil distillate

65 70 fraction, removing the overhead distillate and utilizing the hydrogenated residuum fraction as the tinning oil additive. The residue product is generally referred to in the trade as fatty acid residuum products or fish oil stearine pitches.

75

The pitch can be further split, subjected to distillation, the overhead distillation fraction recovered, hydrogenated and combined with the first overhead distillate product and used as additive products in this invention. Another method of producing the desired distillate fractions is to split the oil first, remove the distillate fraction and then hydrogenate it preferably in the presence of a suitable catalyst and at elevated temperatures.

The overhead distillate products such as described above or those obtained from other fatty oils are not to be confused with the residue products generally referred to as residuum products or pitches. The two fractions are entirely separate and distinct chemically from each other and also from the base oil from which they are derived. As will be hereinafter shown superior results are obtained when hydrogenated fish oil distillates are utilized as tin and metal coating oil additives. However, hydrogenated residuum products derived from fish oils or other hydrogenated fatty oil products can be used for tin-plating oil compositions when in combination with an organic nitrogen-containing stabilizing agent.

Analysis of a hydrogenated marine oil, and its residuum and distillate fractions is given below:

| Properties               | Hydrogenated Marine Oil | Hydrogenated Marine Oil Distillate | Hydrogenated Marine Oil Residuum |
|--------------------------|-------------------------|------------------------------------|----------------------------------|
| Specific Gravity, 60° F. | 0.926                   | 0.950                              | 0.898                            |
| Melting Point, °F.       | 101                     | 145                                | 134                              |
| Acid number              | 1.00                    | 188                                | 149                              |
| Iodine number            | 58.34                   | 3.6                                | 23                               |

Anti-oxidants which are particularly applicable for use with compositions of this invention are high boiling nitrogen containing organic compounds and particularly amine and amine substituted organic compounds having high boiling points. Among the amine compounds which can be included for use in this invention are the aromatic amines, aliphatic amines, alkylaryl amines, cyclic amines, heterocyclic amines and the like and their mixtures. The following amine compounds are applicable as stabilizing agents for metal coating compositions of this invention: paraphenylenediamine, alpha-naphthylamine, orthophenylenediamine, beta-naphthylamine, 5-dibeta-naphthyl para phenylene diamine, 2,4-diamino diphenylamine, meta tolulylene diamine, 2-amino-1,4-naphthohydroquinone, 4-amino-1,2-naphthohydroquinone, thiadiphenylamine, monobenzyl para amino phenyl, 2,4-diamino toluene, 2,4-diamino diphenyl amine, para amino ozobenzene, octadecyl benzyl amine, beta phenylamine-alpha-naphthylamine, phenyl- $\alpha$ -naphthylamine, phenyl- $\beta$ -naphthylamine, N,N'-dibutyl paraphenylenediamine, tetra methyl diamino diphenyl methane, p,p'-diamino diphenyl methane, 4,4-diamino diphenyl methane, tetraethyl diamino diphenyl methane, diisoamyl diamino diphenyl methane, bis-( $\beta$ -naphthyl amine) -p-tertaryl phenol; 3,3,5-tricyclohexylamine, dicyclohexylamine; N-phenyl morpholine, N-(parahydroxyphenyl) morpholine; octadecyl 3-methyl-2-pentylamine, N-octadecyl-2-ethylhexylamine, hexadecylamine, octadecylamine, octadecenylamine, octadecadienyl amine, paraffine waxamine, cocoamine prepared from cocoanut oil acids, N,N'-dimethyl triglycol diamine; disalicyl ethylene diamine; N-salicylal-N'-ethanol-ethylene diamine; 5-methyl, 2,4-di-

amino anisole; ketone diarylamine, ketone amine; ketone amine condensation products; butyraldehyde aniline derivatives; condensation products of acetone and aniline, reaction products of acetone and para amino diphenyl. In addition to the above amine compounds the following mixtures of amines produce good stabilizers. Mixtures of diphenyl paraphenylenediamine and isopropoxydiphenylamine, phenyl- $\alpha$ -naphthylamine and meta tolulylene diamine, mixture of diphenyl para phenylene diamine and para phenylene diamine, mixture of stearic acid, meta tolulylene diamine and phenyl- $\alpha$ -naphthylamine, mixture of ditolylamine and petroleum wax and the like. The amines which are particularly preferred are: phenyl- $\alpha$ -naphthylamine, phenyl- $\beta$ -naphthylamine, beta phenyl-amine- $\alpha$ -naphthylamine, tetra methyl diamino diphenyl methane, meta tolulylene diamine, their mixtures and amines having a boiling point of or above that of phenyl- $\alpha$ -naphthylamine, although this is not a critical limitation but a desirable one.

The addition of nitrogen-containing organic compounds to oil compositions of this invention in addition to inhibiting the oxidation tendencies of the composition greatly improves its tinning properties and stability. In addition it decreases the loss of acid from the oil, reduces the viscosity and improves the draining of the oil from the tin plate.

The mineral oil base used can be any suitable refined petroleum hydrocarbon stock having high flash and fire points and which are substantially stable at tinning temperatures of between about 460-490° F. Suitable petroleum hydrocarbon base stocks which can be used are solvent extracted Mid-Continent Bright stock, acid treated Mid-Continent Bright stock, acid treated naphthenic neutral stock and blends of these oil stocks. Preferably, however, solvent extracted Mid-Continent Bright stock having a Saybolt Universal viscosity at 210° F. of 150-170 is used as the oil base stock because of the superior tinplating results obtained when using this type of oil.

To more fully and clearly illustrate this invention a series of comparative tinning tests were conducted in which the tinning performance as to flux removal, drainage characteristic, ease of cleaning and spreadability characteristics of the following oil compositions were compared:

Code No.

1. Mineral oil (solvent extracted Mid-Continent oil, 150-170 SUS at 212° F.).
2. Palm oil.
3. 20-50% by wt. of palm oil in mineral oil base.
4. Mixture of hydrogenated cottonseed oil in mineral oil base having an acid number of less than 3.
5. Mixture of hydrogenated fish oil residuum or stearine pitches in mineral oil having an acid number of 3 to 15.
6. Mixture of hydrogenated fish oil residuum or stearine pitches in mineral oil having an acid number of 3 to 15 and containing about 0.5% by wt. of phenyl- $\alpha$ -naphthylamine.
7. Mixture of hydrogenated fish oil distillate in mineral oil having an acid number of 3 to 15.
8. Mixture of hydrogenated fish oil distillates in mineral oil having an acid number of 3

- to 15 and containing about 0.5% by wt. of phenyl- $\alpha$ -naphthylamine.
9. Mixture of hydrogenated fish oil distillates in mineral oil having an acid number of 3 to 15 and containing about 0.5% by wt. of tetra methyl diamino diphenyl methane.

One test was conducted as follows:

A. Pickled sheets of black plate, stored in 0.5 per cent HCl, were dipped in flux (3 pounds ZnCl<sub>2</sub> plus 5 ounces NH<sub>4</sub>Cl per gallon) and tinned at temperatures between about 530 and about 560° F., and preferably at 550° F. The tinning pot surface was covered with flux. Sheets were tinned so that very little, if any, flux adhered to the sheets upon withdrawal. Immediately after withdrawal, the sheets were transferred to a finishing pot containing tin at about 530-545° F. and a superimposed layer of oil at about 460-490° F. and preferably at 470° F. The relatively high temperature was necessary to maintain the desired oil temperature. Here the sheets were immersed in the tin and then drained in the oil layer. The metal sheets were immersed in the tin and then drained in the oil layer. Metal strips tested were given a tinning and oil treatment at regular intervals and the test was conducted for a period of 72 hours. The properties as indicated in Table I were graded in descending order, (1) being the best, (2) next best, etc. The results of the test were as follows:

B. Another test was conducted in which the tinning technic was slightly modified. Two tinning pots were used as before, and the temperature of the first tin pot was kept at 535° F. and the final pot at 475° F. Instead of the oil layer on the second pot, a small amount of tallow just sufficient to form a ring covering the bath edges was used to keep the surface clean. Immediately upon withdrawal of the sheet from the second pot, it was transferred to an oil pot kept at a temperature of 460-475° F. To simulate the oil-tin interface encountered in tinplate manufacture, a small amount of tin was poured into the bottom of the oil pot. Tests were conducted for a 72 hour period with the same compositions as indicated in Table I and the results were substantially the same as indicated in Table I.

C. Still another test was conducted in a small tinning machine similar to that described in columns 1 and 2. The tin was melted, put in the oil pot and the flux and oil tested put in the feed and end or exit compartments of the machine respectively. The oil temperature was kept in the range of 475-490° F. Approximately three tests with each oil were conducted during a 24 hour interval and the tinning performance of the oils as to flux removal, draining characteristics, ease of cleaning and spreading characteristics were noted. The results again were similar to those disclosed in Table I, showing the superiority of mineral oil-hydrogenated fish oil distillates over oils tested as a tinning oil.

D. Tests were conducted according to pro-

TABLE I

| Code No.                           | Flux Removal                                  | Draining Characteristics                                                             | Ease of Cleaning                                              | Spreading Characteristics                           | Total | Remarks                                                                                                                                                                                                                                                                                                                                                                                                            |
|------------------------------------|-----------------------------------------------|--------------------------------------------------------------------------------------|---------------------------------------------------------------|-----------------------------------------------------|-------|--------------------------------------------------------------------------------------------------------------------------------------------------------------------------------------------------------------------------------------------------------------------------------------------------------------------------------------------------------------------------------------------------------------------|
| 1.                                 | 10. Poor flux removal.                        | 10. Streaked badly.                                                                  | 10. Flux spots, stained, sticky and difficult to clean.       | 10. Stained, stripped, heavy tinned.                | 40    | Mineral alone was found totally unsatisfactory. At the end of 24 hours sludge formations were high and losses heavy so that test had to be discontinued.                                                                                                                                                                                                                                                           |
| 2.                                 | 3. Showed good flux removal for 72 hour test. | 5. Good draining characteristics for early part of test but streaked after 48 hours. | 4. Easy but flux spots noted.                                 | 3. Good at early stage but spangled about 24 hours. | 15    | Although the tinning characteristic of palm oil were good for 24 hours, oil losses were heavy at the end of the 72 hour test.                                                                                                                                                                                                                                                                                      |
| 3. (30 % Palm oil in mineral oil): | 6. -----                                      | 8. Poor throughout test period.                                                      | 8. Easy to remove but flux spots noted.                       | 7. Stained -----                                    | 20    | After 24 hours the tin plate was stained and spangled. Stripping was noted and draining was poor throughout test. At the end of 24 hours test was discontinued.                                                                                                                                                                                                                                                    |
| 4.                                 | 6. -----                                      | 10. Streaked badly.                                                                  | 8. Stained and difficult to clean.                            | 10. Stained, tinning not very uniform.              | 34    | After a short period the oil was found to be unsatisfactory and test was discontinued.                                                                                                                                                                                                                                                                                                                             |
| 5.                                 | 3. -----                                      | 8. Poor throughout test period.                                                      | 8. Good draining early period of test but became worse later. | 4. Fair -----                                       | 21    | Flux removal and spreading were good. Draining and cleaning were poor and became increasingly worse.                                                                                                                                                                                                                                                                                                               |
| 6.                                 | 3. Good flux removal for 72 hours.            | 5. Good draining at first but became worse as test continued.                        | 3. Good -----                                                 | 3. Good at beginning of test but left stains.       | 14    | The addition of the amine antioxidant resulted in a product equivalent to or superior to palm oil.                                                                                                                                                                                                                                                                                                                 |
| 7.                                 | 1. Good -----                                 | 3. Good for 48 hours, but at end of test period showed signs of poor draining.       | 3. Same -----                                                 | 2. Good -----                                       | 10    | Flux removal and spreading were good. Exhibited a pronounced stabilizing effect on the composition and gave good tinning performance at the end of 48 hours and fair tinning performance at the end of 72 hours. Oil losses were only $\frac{1}{3}$ of that of palm oil after 72 hrs.                                                                                                                              |
| 8.                                 | 1. Very good -----                            | 2. Good for entire 72 hour test.                                                     | 2. Good -----                                                 | 2. Good -----                                       | 7     | Flux removal and spreading were good. Exhibited a pronounced stabilizing effect on the composition and gave good tinning performance for entire 72 hour test period. Oil losses were only $\frac{1}{3}$ of that of palm oil after 72 hours and required 8.8% by wt. less replenishing agent so as to maintain the acid number of the composition between 3 and 15 than was required for composition of Code No. 5. |
| 9.                                 | 1. Very good -----                            | 2. -----                                                                             | 2. -----                                                      | 2. -----                                            | 7     | Flux removal and spreading were good. Exhibited a pronounced stabilizing effect on the composition and gave good tinning performance for entire 72 hour test period. Oil losses were only $\frac{1}{3}$ of that of palm oil after 72 hours and required 8.8% by wt. less replenishing agent so as to maintain the acid number of the composition between 3 and 15 than was required for composition of Code No. 5. |

cedure outlined under A and B in order to determine the criticality of maintaining the acid number of mineral oil-hydrogenated fish oil distillates between about 3 to 15.

To further show the marked effect on oxidation stability nitrogen-containing organic compounds have on tinning oil compositions of this invention the Dornte oxidation test as fully described in the

TABLE II

|                                                                                                                                                          | Flux Removal | Draining Characteristics | Ease of Cleaning | Spreading Characteristics | Total | Remarks                                                                                 |
|----------------------------------------------------------------------------------------------------------------------------------------------------------|--------------|--------------------------|------------------|---------------------------|-------|-----------------------------------------------------------------------------------------|
| 1 Mineral oil-hydrogenated fish oil distillates having an acid number less than 3.                                                                       | 8            | 9                        | 7                | 6                         | 30    | Drained very poorly and unstable.                                                       |
| 2 Mineral oil-hydrogenated fish oil distillates having an acid number greater than 15.                                                                   | 3            | 6                        | 7                | 4                         | 20    | Cause etching of metal surface and difficult to clean.                                  |
| 3 Mineral oil-hydrogenated fish oil distillates having an acid number between about 4-10.                                                                | 2            | 3                        | 3                | 2                         | 10    | Good spreading characteristics and stable.                                              |
| 4 Mixture of mineral oil and hydrogenated fish oil distillates having an acid number of 15 and containing 0.5% wt. phenyl- $\alpha$ -naphthylamine.      | 1            | 2                        | 2                | 2                         | 7     | Flux and draining properties improved and no sludge was noted after a 72 hr. test run.  |
| 5 Mixture of mineral oil and hydrogenated fish oil distillates having an acid number of 15 and containing 0.5% wt. tetra methyl diamino diphenylmethane. | 1            | 2                        | 2                | 2                         | 7     | Flux and draining properties improved and no sludge was noted after a 72 hour test run. |
| 6 Mineral oil-hydrogenated cottonseed oil having an acid number of less than 3 (0.62).                                                                   | 6            | 10                       | 8                | 10                        | 34    | Product unsatisfactory as a tinning composition.                                        |

As has been repeatedly pointed out the acid number of a suitable tinning oil composition must be kept at not less than 3 and not above about 15. Due to the elevated temperatures under which tinning compositions and the like are used the acid number varies and in order to readjust it within the desired acid range a replenishing agent is used. The replenishing agent consists essentially of a concentrated mineral oil and a desired hydrogenated fatty oil or any of its fractions, but preferably the overhead distillate fraction made up in the ratio varying from 1:3 to around about 3:1 parts by weight of each ingredient respectively. Preferably the above ingredients should be mixed in approximately equal parts and is added to the base composition in amounts sufficient to readjust the acid number between about 3 to 15.

A quick and conclusive test was developed to study the draining characteristics of tinning oils. A heavily tinned plate was immersed for 15 seconds into an oil kept at a temperature of approximately 480° F. Heavily tinned plates were repeatedly dipped in the various oils during a 24 hour interval and the characteristics of the oil film remaining on the plate were preserved by printing off on a hard filter paper and observations made.

TABLE III

|                                                                                                                                                            | Composition                                                                                                       |  |
|------------------------------------------------------------------------------------------------------------------------------------------------------------|-------------------------------------------------------------------------------------------------------------------|--|
| 1 Mineral oil                                                                                                                                              | Drained poorly through test period. Filter paper covered with a heavy oil film.                                   |  |
| 2 30% by wt. of Palm oil in mineral oil.                                                                                                                   | Drained poorly, paper covered with an oil film.<br>Do.                                                            |  |
| 3 Mineral oil-hydrogenated fish oil distillates having an acid number less than 3.                                                                         | Drained very well, few oil spots on paper.<br>Equal to, if not superior to, palm oil in draining characteristics. |  |
| 4 Palm Oil                                                                                                                                                 | Drained poorly, paper covered with an oil film.<br>Results similar to palm oil.                                   |  |
| 5 Mineral oil-hydrogenated fish oil distillates having an acid number between 3 and 15.                                                                    | Superior to palm oil in draining characteristics.                                                                 |  |
| 6 Mineral oil-hydrogenated fish oil residuum product having an acid number between 3 and 15.                                                               | Do.                                                                                                               |  |
| 7 Mineral oil-hydrogenated fish oil residuum product having an acid number between 3 and 15 and containing 0.5% by wt. of phenyl- $\alpha$ -naphthylamine. | Drained very poorly during test period.                                                                           |  |
| 8 Mineral oil-hydrogenated fish oil distillates having an acid number between 3 and 15 and containing 0.5% by wt. of phenyl- $\alpha$ -naphthylamine.      |                                                                                                                   |  |
| 9 Composition of 6 but the antioxidant used here is tetra methyl diamino diphenyl methane.                                                                 |                                                                                                                   |  |
| 10 Mineral oil-hydrogenated cottonseed oil having an acid number of less than 3.                                                                           |                                                                                                                   |  |

Industrial Engineering Chemistry of August 1942, volume 34, page 927, was conducted and compared with other tinning oil compositions.

TABLE IV

Dornte Oxidation Test, minutes volume oxygen absorbed, 1800 cc./100 gm. oil 313° F. copper present

|                                                                                                                              |           |          |
|------------------------------------------------------------------------------------------------------------------------------|-----------|----------|
| Per Cent Phenyl- $\alpha$ -naphthylamine added.....                                                                          | None..... | 0.5% wt. |
| Mineral Oil of hydrogenated fish oil distillates in mineral oil having an acid number of 15 (8.0% by wt. of the distillate). | 200.....  | 385.     |

The effect anti-oxidants have on compositions of this invention were further vividly illustrated when hydrogenated fish oil distillates in mineral oil having an acid number of 15 were compared with the same composition but having admixed therein 0.5% by weight phenyl- $\alpha$ -naphthylamine.

The tinning was conducted in the manner described under Test A except that the test was conducted for 216 hours and the oils were kept at a temperature between about 465-485° F. The results are:

| Remarks                                                                                              | Composition <sup>1</sup> and Data |                                                |
|------------------------------------------------------------------------------------------------------|-----------------------------------|------------------------------------------------|
|                                                                                                      | Code No. 7                        | Code No. 8                                     |
| Amount of replenishing agent required during test period in order to maintain the acid number at 15. | -----                             | 8.8% by wt. less than that used in Code No. 7. |

<sup>1</sup> 7 and 8 are the same composition as referred to in Table I.

Viscosity changes in the compositions after the following number of test hours (S. U. S. at 210° F.):

| Hours  | Viscosity changes for Code No. 7 | Viscosity changes for Code No. 8 |
|--------|----------------------------------|----------------------------------|
| 0.33   | 143.2                            | 141.0                            |
| 73.00  | 219.1                            | 194.2                            |
| 151.50 | 338.8                            | 260.4                            |
| 215    | 503.2                            | 317.6                            |

The anti-oxidants phenyl- $\alpha$ -naphthylamine and tetra methyl diamino diphenyl methane were only used for illustrative purposes in the above tests and these are not to be construed as limitations of this invention. Other amines listed herein are also applicable for purposes of this invention giving improved tinning results.

Modifications as to procedure of tinning and

## 11

composition can be made in order to obtain an improved tinplate with the use of composition of this invention. Thus, minor amounts of high molecular fatty acids such as oleic, stearic and the like can be added to compositions of this invention to improve the lustre of the tinplate, and spreadability of the tinning composition. Also non-hydrogenated animal and vegetable oils such as cocoanut oil, castor oil, cottonseed oil, peanut oil and the like as well as synthetic lubricants produced by polymerization of olefins can be admixed with composition of this invention.

Compositions of this invention are not restricted to use in tinplating only but are equally applicable for terne coating, lead coating and the like. Neither are these compositions restricted to use where metal plating is done only by dipping and the like. Compositions of this invention can be used to improve the metal coating surface and deposition of metals on metal base by electrolytic methods as well as any other known metal plating method. The appearance of surfaces having tin deposited thereon by electrolytic means is greatly improved by dipping such metal treated surfaces into a hot bath comprising an oil composition of this invention.

In addition to being equal to and in most properties superior to palm oil, compositions of this invention have a particular advantage over palm oil in that they reduce to a minimum the danger of fire hazard.

It is to be understood that while the features of the invention have been described and illustrated in connection with specific compositions, the invention is not limited thereto or otherwise restricted, except by the prior art and the scope of the appended claims.

I claim as my invention:

1. In a method of tin coating a metal surface wherein a metal is cleaned and pickled and wherein said cleaned metal is passed through a flux bath consisting essentially of a zinc chloride-ammonium chloride solution, followed by passing the metal into a molten tin bath maintained at a temperature or between about 530° and about 560° F., and passing said tin-treated metal through an oil composition maintained at a temperature of between about 460° and about 500° F., the improvement residing in using as said oil composition a mixture consisting essentially of mineral oil and partially hydrogenated fish oil distillates, said mixture having an acid number of not less than 3 and not more than about 15, and containing a minor amount sufficient to stabilize the composition against deterioration of phenyl-*α*-naphthylamine.

2. In a method of tin coating a metal surface wherein a metal is cleaned and pickled and wherein said cleaned metal is passed through a flux bath consisting essentially of zinc chloride-ammonium chloride solution, followed by passing the metal into a molten tin bath maintained at a temperature of between about 530° and about 560° F. and passing said tin treated metal through an oil composition maintained at a temperature of between about 460° and about 500° F., the improvement residing in using as said oil composition a mixture consisting essentially of mineral oil and partially hydrogenated fish oil distillates, said mixture having an acid number of not less than 3 and not more than about 15 and containing a minor amount sufficient to stabilize the composition against deterioration of tetra methyl diphenyl methane.

3. In a method of tin coating a metal surface

## 12

wherein a metal is cleaned and pickled and wherein said cleaned metal is passed through a flux bath consisting essentially of a zinc chloride-ammonium chloride solution, followed by passing the metal into a molten tin bath maintained at a temperature of between about 530° and about 560° F. and finally passing said tin treated metal through an oil composition maintained at a temperature of between about 460° and about 500° F. the improvement residing in using as said oil composition a mixture consisting essentially of mineral oil and partially hydrogenated fish oil distillates, said mixture having an acid number of not less than 3 and not more than about 15 and containing a minor amount sufficient to stabilize the composition against deterioration of meta tolulylene diamine.

4. In a method of tin coating a metal surface wherein a metal is cleaned and pickled and wherein said cleaned metal is passed through a flux bath consisting essentially of a zinc chloride-ammonium chloride solution, followed by passing the metal into a molten tin bath maintained at a temperature of between about 530° and about 560° F. and finally passing said tin treated metal through an oil composition maintained at a temperature of between about 460° and about 400° F. the improvement residing in using as said oil composition a mixture consisting essentially of mineral oil and partially hydrogenated fish oil distillates, said mixture having an acid number of not less than 3 and not more than about 15 and containing a minor amount sufficient to stabilize the composition against deterioration of a high boiling unsubstituted hydrocarbon amine.

5. In a method of metal coating a metal surface of a base metal wherein said base metal is cleaned and pickled and wherein said cleaned metal is passed through a flux bath, on through a molten metal bath selected from the class consisting of molten tin, molten lead and a molten metal mixture of lead and tin, and finally passing said metal through an oil composition, maintained at an elevated temperature, the improvement residing in using as said oil composition a blend consisting essentially of mineral oil and partially hydrogenated fish oil and marine oil distillates, said blend having an acid number of not less than 3 and not more than about 15, and containing a minor amount sufficient to stabilize the composition against deterioration of a high boiling unsubstituted aryl amine.

6. In a method of metal coating a metal surface of a base metal wherein said base metal is cleaned and pickled and wherein said cleaned metal is passed through a flux bath, on through a molten bath selected from the class consisting of molten tin, molten lead and a molten metal mixture of lead and tin, and finally passing said metal through an oil composition, maintained at an elevated temperature, the improvement residing in using as said oil composition a blend consisting essentially of mineral oil and partially hydrogenated fish oil and marine oil distillates, said blend having an acid number of not less than 3 and not more than about 15, and containing a minor amount sufficient to stabilize the composition against deterioration of a high boiling unsubstituted hydrocarbon amine.

7. In a method of tin coating a metal surface wherein a metal is cleaned and pickled and wherein said cleaned metal is passed through a flux bath consisting essentially of a zinc chloride-ammonium chloride solution, followed by passing the metal into a molten tin bath maintained

at a temperature of between about 530° and about 560° F. and finally passing said tin treated metal through an oil composition, maintained at a temperature of between about 460° and about 490° F., the improvement residing in using as said oil composition a mixture of mineral oil and partially hydrogenated fish oil distillates and a minor amount sufficient to stabilize the composition against deterioration of a high boiling unsubstituted aryl amine, said oil composition being replenished at intervals with a concentrate comprising approximately equal parts of a mixture of hydrogenated fish oil distillates and mineral oil, in amounts sufficient to maintain the acid number of said oil composition between about 3 to 15.

8. In a method of metal coating metal surfaces wherein a metal is cleaned and pickled and wherein said cleaned metal is passed through a flux metal bath, on through a molten metal bath selected from the class consisting of molten tin, molten lead and mixtures of molten lead and tin and finally passing said metal through an oil composition, maintained at an elevated temperature, the improvement residing in using as said oil composition a blend consisting essentially of mineral oil and partially hydrogenated fish oil distillates, containing a minor amount sufficient to stabilize the composition against deterioration of a high boiling unsubstituted aryl amine, said composition being replenished at intervals with a concentrate comprising approximately equal parts of a mixture of hydrogenated fish oil distillates and mineral oil, in amounts sufficient to maintain the acid number of said composition between about 3 to 15.

9. In a method of metal coating metal surfaces wherein a metal is cleaned and pickled and wherein said cleaned metal is passed through a flux bath, on through a molten bath selected from the class consisting of molten tin, molten lead and a molten metal mixture of lead and tin, and finally passing said metal through an oil composition, maintained at an elevated temperature, the improvement residing in using as said oil composition a blend consisting essentially of mineral oil and a hydrogenated fatty oil selected from the class consisting of hydrogenated animal, vegetable, marine oils, hydrogenated residuum fractions of said oils and hydrogenated distillate fractions of said oils, said blend having an acid number of not less than 3 and not more than about 15 and containing a minor amount sufficient to stabilize the composition against deterioration of a high boiling unsubstituted aryl amine.

10. In a method of tin coating metal surfaces wherein a metal is cleaned and pickled and wherein said cleaned metal is passed through a flux bath consisting essentially of a zinc chloride-ammonium chloride solution, followed by passing the metal into a molten tin bath maintained at a temperature of between about 530° and about 560° F. and finally passing said tin treated metal through an oil composition, maintained at a temperature of between about 460 and about 490° F., the improvement residing in using as said oil composition a blend consisting essentially of mineral oil and hydrogenated fatty oil, said blend having an acid number of not less than 3 and not more than about 15, and containing a minor amount sufficient to stabilize the composition against deterioration of a high boiling unsubstituted aryl amine.

11. In a process of aiding in forming an adherent tin coating on ferrous surfaces the step

of contacting said tin coated surface with a composition consisting essentially of an oil blend of mineral oil and partially hydrogenated fish oil distillates and a minor amount sufficient to stabilize the composition against deterioration of phenyl-*a*-naphthylamine, said composition having an acid number of between about 3 and 15.

12. In a process of aiding in forming an adherent tin coating on ferrous surfaces, the step of contacting said tin coated surface with a composition consisting essentially of an oil blend of mineral oil and partially hydrogenated fish oil distillates and a minor amount sufficient to stabilize the composition against deterioration of tetramethyl diamine-diphenyl methane, said composition having an acid number of between about 3 and 15.

13. In a process of aiding in forming an adherent tin coating on ferrous surfaces, the step of contacting said tin coated surface with a composition consisting essentially of an oil blend of mineral oil and partially hydrogenated fish oil distillates and a minor amount sufficient to stabilize the composition against deterioration of meta tolulylene diamine, said composition having an acid number of between about 3 and 15.

14. In a process of aiding in forming an adherent tin coating on ferrous surfaces, the step of contacting said tin coated surface with a composition consisting essentially of an oil blend of mineral oil and partially hydrogenated fish oil distillates and a minor amount sufficient to stabilize the composition against deterioration of a high boiling unsubstituted hydrocarbon amine, said composition having an acid number of between about 3 and 15.

15. In a process of aiding in forming an adherent metal coating on ferrous surfaces, the step of contacting said tin coated surface with a composition consisting essentially of a mixture of mineral oil and partially hydrogenated fish oil distillates and a minor amount sufficient to stabilize the composition against deterioration of a high boiling unsubstituted hydrocarbon amine, said composition being replenished during use with a concentrate comprising approximately equal parts of a mixture of hydrogenated fish oil distillates-mineral oil, in amounts sufficient to maintain the acid number of said composition between about 3 to 15.

16. A mineral oil composition suitable for aiding in the formation of an adherent coating on ferrous surfaces with molten metals selected from the class consisting of tin, lead and mixtures of tin and lead, consisting essentially of a blend of mineral oil and partially hydrogenated fish oil distillates and a minor amount sufficient to stabilize the composition against deterioration of a high boiling unsubstituted aryl amine, said composition having an acid number of between about 3 to 15.

17. A mineral oil composition suitable for aiding in the formation of an adherent tin coating on ferrous surfaces, consisting essentially of a blend of mineral oil and hydrogenated fatty oil and a minor amount sufficient to stabilize the composition against deterioration of a high boiling unsubstituted aryl amine, said composition having an acid number of between about 3 to 15.

18. A mineral oil composition suitable for aiding in the formation of an adherent tin coating on ferrous surfaces, consisting essentially of a blend of mineral oil and a hydrogenated fatty oil selected from the class consisting of hydrogenated animal, vegetable and marine oils, hydrogenated

residuum fractions of said oils and hydrogenated distillate fractions of said oils and a minor amount sufficient to stabilize the composition against deterioration of a high boiling unsubstituted hydrocarbon amine said composition having an acid number of between about 3 to 15.

19. A mineral oil composition suitable for aiding in the formation of an adherent coating on ferrous surfaces with molten metals selected from the class consisting of tin, lead and mixtures of tin and lead, consisting of a blend of mineral oil and partially hydrogenated fish oil distillates and a minor amount sufficient to stabilize the composition against deterioration of a high boiling unsubstituted aryl amine, said composition having an acid number of between about 3 to 15.

20. A mineral oil composition suitable for aiding in the formation of an adherent coating on ferrous surfaces with molten metals selected from the class consisting of tin, lead and mixtures of tin and lead, consisting of a blend of mineral oil and partially hydrogenated fish oil distillates and from 0.25% to 2% sufficient to stabilize the composition against deterioration of a high boiling unsubstituted aryl amine, said composition having an acid number of between about 3 to 15.

21. A mineral oil composition suitable for aiding in the formation of an adherent coating on ferrous surfaces with molten metals selected from the class consisting of tin, lead and mixtures of tin and lead, a blend consisting essentially of mineral oil and a hydrogenated fatty oil, said blend having an acid number of between 3 and 15 and containing a minor amount sufficient to stabilize the composition against deterioration of a high boiling unsubstituted hydrocarbon amine.

22. A mineral oil composition suitable for coating on ferrous surface with molten tin, a blend consisting essentially of mineral oil and hydrogenated fish oil distillate having an acid number of between 3 and 15 and containing phenyl-naphthyl amine in an amount sufficient to prevent deterioration of said blend.

GEORGE W. WATERS.

10

#### REFERENCES CITED

The following references are of record in the file of this patent:

#### UNITED STATES PATENTS

| 15 | Number    | Name             | Date          |
|----|-----------|------------------|---------------|
|    | 1,829,999 | Merkle           | Nov. 3, 1931  |
|    | 1,998,767 | MacLaren         | Apr. 23, 1935 |
|    | 2,044,210 | Gordon           | June 16, 1936 |
|    | 2,062,675 | Rather et al.    | Dec. 1, 1936  |
| 20 | 2,099,236 | Sibley           | Nov. 16, 1937 |
|    | 2,229,368 | Brunstrom et al. | Jan. 21, 1941 |
|    | 2,270,577 | Bergstrom        | Jan. 20, 1942 |
|    | 2,291,460 | Francis          | July 28, 1942 |
|    | 2,298,640 | Prutton          | Oct. 13, 1942 |
| 25 | 2,356,863 | MacLaren et al.  | Aug. 29, 1944 |
|    | 2,362,332 | Zimmer et al.    | Nov. 7, 1944  |
|    | 2,451,642 | Watson           | Oct. 19, 1948 |

#### OTHER REFERENCES

30 Oil, Paint and Drug Reporter, October 23, 1939, page 52.

Oil, Paint and Drug Reporter, October 30, 1939, page 30.